

# UNITED STATES PATENT OFFICE.

JEAN A. HARDEL, OF PARIS, FRANCE.

## EXPLOSIVE.

1,337,451.

Specification of Letters Patent. Patented Apr. 20, 1920.

No Drawing.

Application filed February 4, 1919. Serial No. 275,008.

To all whom it may concern:

Be it known that I, JEAN AMÉDÉE HARDEL, a citizen of the Republic of France, residing at Paris, France, have invented a certain new and useful Improvement in Explosives, of which the following is a specification.

My invention relates to explosives and particularly to an explosive mixture comprising a plurality of elements each safe to handle independently, but which when combined form a rapid explosive of great power and efficiency and having a further characteristic that the chemical reaction which occurs after the mingling of the elements renders the explosive innocuous after the lapse of a few hours.

It is frequently the case, and especially in operations at mines, quarries, and oil wells, that it would be advantageous to substitute for ordinary explosives, an explosive, the elements of which are not mingled until the moment at which the explosive charge is to be utilized. The transportation of dangerous materials is thus avoided. However, a satisfactory explosive of this character has not hitherto been proposed although certain explosives of this general type have already been suggested.

The first type of explosive having this general characteristic consists of the so called "panclastites" composed of nitrogen peroxid to which is added, at the moment of explosion, a combustible such as a hydrocarbon (gasolene) or a substance previously nitrated (dynamite). But nitrogen peroxid is not a commercial product and is moreover a rather delicate substance having a very low boiling point (21° C.—70° F.), a fact which renders its use difficult under the common condition of higher temperatures and by reason of the further fact that its vapors are extremely noxious.

A second type of explosive having the general characteristic above referred to, consists of a mixture of pure nitric acid (approaching as closely as possible the formula  $\text{NO}_3\text{H}$ ) with mono-, di-, or tri-nitro derivatives of benzine or its homologues, and especially of toluene. The mixtures with the di- or tri-nitro derivatives afford satisfactory explosives, but these derivatives are solid at ordinary temperatures, and moreover for the handling of these explosives, which must be completely protected against moisture, and mixed in a closed container at the place

of use, it is more difficult to make a satisfactory container when the mixture comprises a solid and a liquid separately housed, than for two liquids. Furthermore, the weight of a solid product contained within a chamber of given volume is reduced by the voids in the solid and the explosive power of the charge is thus to a certain extent reduced. The mono-nitro derivatives, which are liquid, afford an explosive of much lower power than the higher nitro derivatives, and are of such instability that they are quite subject to spontaneous combustion. These derivatives, therefore, while less dangerous in the sense that they may be employed in an explosive mixture made at the place of use, may nevertheless be quite dangerous under certain conditions and present serious difficulties from the technical stand-point.

I have now discovered that a satisfactory explosive may be obtained by mixing pure nitric acid with a liquid solution of di- or tri-nitro derivatives in a mono-nitro derivative. My experiments have demonstrated that an explosive of this character is entirely satisfactory. The power of the explosive is greater than that of nitroglycerin, for equal volumes. The speed of detonation is thrice as great as that of nitroglycerin—a fact which renders the explosive more shattering in its effect. The mixture with nitric acid is made without danger and without marked rise of temperature.

Various mixtures are contemplated in forming the solution of di- or tri-nitro derivatives in the mono-nitro derivative, the sole condition being that the eutectic mixture thus constituted shall be liquid and that it shall comprise the lowest possible percentage of mono-nitro derivative and the greatest possible percentage of di- or tri-nitro derivatives. As an example, the following formula may be recommended:

|                        |                       |
|------------------------|-----------------------|
| Di-nitro-benzin.....   | 100 parts (by weight) |
| Di-nitro-toluene.....  | 100 " " "             |
| Mono-nitro-benzin..... | 50 " " "              |

250 parts to be mixed with

450 parts.

With equal facility, it is possible to incorporate tri-nitro-toluene in the mixture. Such a mixture is very rich in  $\text{NO}_2$  and after mingling with a suitable proportion of nitric acid affords an explosive of great shattering power by reason of the speed of detonation.

The containers to be employed in handling

this explosive may be merely sheet steel which is not attacked by either pure nitric acid or the mixtures of nitro derivatives.

An important advantage in an explosive 5 of this composition is that after the mixture with nitric acid has been effected, a slow progressive nitration occurs which is accompanied by the formation of water. As a result, if the mixture is not speedily detonated for any reason, such for instance as the breakage of the wire which carries the current to the electric detonator, or the failure of the cap of an ordinary detonator, the charge 10 may be removed without danger after the lapse of a few hours in which time sufficient water has been formed to render the explosive mixture innocuous. It is of course intended that the detonation of the explosive mixture should follow immediately after the 15 mingling of the nitro derivatives with nitric acid has been effected, and this presents no difficulty since it is possible by the use of suitable arrangements to effect the ignition when desired. A suitable apparatus of this 20 type is disclosed in my co-pending application Serial No. 253,407 relating to oil well 25 torpedoes.

While I have referred above to the use of pure nitric acid, I do not wish to be understood to mean absolutely pure acid. It suffices for the purpose of the mixture to use commercial nitric acid of a density greater than 1.49 and containing preferably not more than from 2% to 5% of water. No 30 doubt other hydrocarbon derivatives than those above mentioned may be successfully employed although those mentioned are the most satisfactory now known to me. Various other combinations and modifications of 35 the underlying thoughts of my discovery will readily occur to those skilled in the art without departing from what I claim as my 40 invention.

I claim—

1. As an element of an explosive mixture, 45 a compound of mono- and higher nitro-hydrocarbon derivatives, said compound being liquid at ordinary temperatures and comprising less than 25% of the mono-hydrocarbon derivative.
2. As an element of an explosive mixture, 50 a solution of mono- and higher nitro-hydrocarbon derivatives, the mono-hydrocarbon derivative constituting less than 25% of the solution.
3. As an element of an explosive mixture, 55 a normally liquid nitro hydrocarbon derivative approximately saturated with a normally solid hydrocarbon nitro-derivative.
4. An explosive comprising a mixture of 60 nitric acid and hydrocarbon nitro-derivatives in which slow nitration accompanied by the formation of water occurs.
5. As an element of an explosive mixture, 65 a liquid comprising a solution of mono- and higher nitro-benzin derivatives, the mono-nitro-benzin constituting less than 25% of the solution.
6. An explosive comprising nitric acid 70 mixed with a solution of a higher nitro-benzin derivative in a mono-nitro-benzin derivative.
7. As an element of an explosive mixture with nitric acid, a liquid comprising a eutectic mixture of mono and higher nitro 75 hydrocarbon derivatives.
8. As an element of an explosive mixture with nitric acid, a liquid comprising a eutectic mixture of mono and higher nitro hydrocarbon derivatives, the mono derivative being present only in sufficient quantity to effect solution.

In testimony whereof I have signed my name to this specification.

JEAN A. HARDEL.